# EUROPEAN PATENT APPLICATION

(11) **EP 0 058 262 A1**
(43) Date of publication of application: **25.08.1982**
(21) Application number: 81300614.5
(22) Date of filing: 13.02.1981
(51) Int. Cl.: B41M 5/12

(54) **Developing sheet for carbonless reproduction paper**

(71) Applicant: Mitsubishi Paper Mills, Ltd., Chiyoda-ku, Tokyo (JP)
(72) Inventor: Nagayasu, Isao, Himeji-shi Hyogo-ken (JP); Toyama, Koji, Katsushika-ku Tokyo (JP)
(74) Representative: Farwell, William Robert

(57) **Abstract**

A developer sheet for carbonless reproduction paper having a phenolic resin developer comprising an ammonium salt of an organic or inorganic acid as an anti-yellowing agent. Desirably the developer further comprises an activated clay.

## Description

### OUTLINE

(1) The present invention relates to a carbonless reproduction paper which features the following. That is; such a developer sheet for carbonless reproduction paper uses a phenolic resin developer comprising as an additive an ammonium salt of an organic or inorganic acid.
(2) The present invention further relates to a carbonless reproduction paper as described in point 1 which has the following features. That is; the phenolic resin developer comprises an activated clay.
(3) The present invention further relates to a carbonless reproduction paper as described in point 1 which has the following features. That is; it uses 1 - 300 wt. parts of ammonium salt as against 100 wt. parts of phenolic resin.

### DETAILED DESCRIPTION OF THE PRESENT INVENTION:

The present invention relates to a developer sheet for carbonless reproduction paper, further detailedly to a developer sheet which features the following. That is; that it uses phenolic resin or phenolic resin with activated clay,as developer, characterised in that an ammonium salt is present in it. So-called carbonless paper has been publicly known and as described for example in the U.S. Patent Specification Nos. 2 712 507, 2 730 465 and 2 730 457it utilizes both microcapsules containing a solution in an organic solvent of a colorless organic compound (hereinafter referred to as coupler) having electron donating adsorbable coloring reactive property and an electron accepting reactive adsorbing substance (hereinafter referred to as developer). Hitherto, microcapsules have been manufactured through various methods for example, such as the coacervation method, the interfacial polymerization method, the in situ method and so on, and as coupler melachite green lactone, crystal violet lactone, benzoyl leuco methylene blue, rhodamine-B-lactam, 3-dialkyl amino-7-dialkyl amyl fluorane, 3-methyl-2, 2-spiropy (benzo-(f)-chromen) and so on, has been used. Further, as the aforementioned developer inorganic developers such as activated clay, acid clay, attapulguite, zeolite, bentonite and the like, and organic compounds for example phenolic resin such as para-tertiary butyl phenolic resin, paraphenyl phenolic resin and so on or succinic acid, tannic acid, maloic acid, maleic acid, gallic acid and the like, further aromatic carboxylic acid such as benzoic acid, salicylic acid, substituted salicylic acid, naphthoeic acid, diphenic acid and so on or metallic acids of these have been well known among those concerned. Such a developer sheet that uses phenolic resin out of these developers is so constructed that it shows good coupling property and excellent color fastness of coupled characters, and generally it has been widely used, but it has such defects in that it shows deteriorated yellowing property and weather resistance (particularly, yellowing property due to ultraviolet ray irradiation) of white part of developer sheet due to adsorption of nitrogen oxidant (NOₓ) in the atmospheric air. Further, in recent years, as described in the Patent Publication No. SHO 50-17888 Japan combined use of phenolic resin and solid acid has come to be prevalent, but in this case further such a defect that it is likely to turn out yellowing has become outstanding and the need for improvement has been urgently studied.

The object of the present invention is to provide such a developer sheet for carbonlessreproduction paper, that is, to improve yellowing property due to adsorption of nitrogen oxidant present in the atmospheric acid and weather resistance, particularly yellowing property due to the effect of ultraviolet rays. In case of the former it takes effect corresponding to preserving resistance in a dark place, while in case of the latter it corresponds to preserving resistance in a bright place so that both may be factors having significant meaning for commercial value of paper. The inventors of the present invention have found that the aforementioned object can be attained by adding ammonium salt of acid into the system using at least phenolic resin as developer. Particularly remarkable effects can be observed in case of a system combinedly using phenolic resin and solic acid, especially activated clay.

What is called ammonium salt of acid that can be used for the present invention includes for example, organic acid ammonium salts such as ammonium acetate, ammonium alginate, n-ammonium butyrate, ammonium oxalate, ammonium dicitrate, ammonium tricitrate, ammonium ditartrate, ammonium succinate, ammonium lactate, ammonium adipate, ammonium sebacinate, ammonium phthalate, ammonium benzoate and so on and inorganic acid ammonium salts such as ammonium chloride, ammonium sulfate, ammonium nitrate, ammonium carbonate, ammonium thiosulfate, ammonium hydrogen sulfate, ammonium persulfate, ammonium phosphate, ammonium diphosphate, ammonium triphosphate and so on. These can be singularly or combinedly used, and among these as particularly favorable examples ammonium phthalate, ammonium citrate, ammonium sulfate, ammonium phosphate and ammonium chloride can be cited.

The amount of ammonium salts of these acids is 1 - 300 wt. parts as against 100 wt. parts of phenolic resin, especially favorable 30 - 120 wt. parts. In case of using below 1 part of the above compound sufficient effect may not be raised, and even in case of more than 300 parts remarkable effect may not be shown, and in addition there are some cases where it tends to impair liquid property and coupling property. However, in this case method of adding these ammonium salts of acids is not particularly restricted. Phenolic resins that can be used for the present invention include paraphenyl phenolic resin, para-tertiary butyl phenolic resin, pera-octyl phenolic resin, parachlor phenolic resin, paracumyl phenolic resin, metal salts of these (Zu, Mg etc) and so on, but from the viewpoint of coupling property and color-fading property of coupled characters it is particularly desirable to use para-phenyl phenolic resin.

Moreover, activated clay that can be used in the system where it is used with phenolic resin is so constructed that acid clay or similar clays are treated with mineral acid so that alumina, iron and any other basic component soluble in acid may be deposited until its surface area shows more than 200m²/g, but in this case it little matters whether metal salts of zinc, magnesium and so on are mixed in it. As binder used for the present invention starch, dextrine, casein, gum arabic, styrene-butadiene latex, butadiene- acrylnitrile latex, vinyl acetate latex, polyvinyl alcohol and the like can be used without being particularly restricted. As material for it the suitable amount of inorganic pigments such as calcium carbonate, zinc oxide, kaolin, clay and so on and organic pigments such as urea- formalin resin micropowder and so on is used.

Together with the aforementioned pigment, binder and so on phenolic resin and acid ammonium salt are used so that coating liquid may be prepared, and then coating liquid is coated on base material such as paper in such a way that developer sheet can be obtained. Further, after developer sheet is produced through any ordinary method by overcoating acid ammonium salt on it the same effect as described above can be obtained.

Kicrocapsules containing coupler can be manufactured for example according to the U.S. Patent Specification No.2 800 457, and its concrete example will be concretely described as follows. After microcapsules containing coupler are dissolved in 100 wt. parts (hereinafter the term "Part" referred to as weight part) in which 2 parts of crystal violet lactone and 1 part of benzoyl leuco methylene blue are dissolved, solution thus obtained is emulsified in 160 parts of acid-treated gelatine (isoelectric point 7.8) 10% aqueous solution. Emulsion thus obtained is added with solution obtained by dissolving 20 parts of gum arabic into 1500 parts of water until pH is adjusted to 3.5. While keeping the liquid temperature to 50°C pH is adjusted to 4.4 with acetic acid and cooled to 10°C and added with 20 parts of 37% formalin aqueous solution and kept being stirred over the night, and then pH is adjusted to 10 with caustic soda so that microcapsules liquid containing coupler can be obtained.

Coupler sheet is obtained through the following method. 50 parts of 10% starch oxide aqueous solution and 30 parts of wheat starch granules are added into 100 parts (solid content) of microcapsules containing coupler and then coated on quality paper of 40 g by means of air knife coater so that the coating amount may indicate 5 g/m²(solid content).

### (MANUFACTURE OF DEVELOPER SHEET FOR CARBONLESS REPRODUCTION PAPER)

### EXAMPLE l:

After as pigment 100 parts of heavy calcium carbonate is gently added into 100 parts of aqueous solution in which 0.5 part of sodium pyrophosphate is dissolved while stirring so that it way be well dispersed, dispersion thus obtained is added with 100 parts of 10% starch oxide aqueous solution, 10 parts (solid content) of SBR latex (Dow 670, manufactured by Dow Chemical Co., Ltd.) and 30 parts of 40% paraphenyl phenolic resin dispersion, and further added with 5 parts of ammonium phthalate so that pH may be adjusted to 9.0 with 20% caustic soda until coating liquid is prepared. Coating liquid is coated on quality paper of 40 g/m² by means of air knife coater so that the coating amount may indicate 7 g/m² (solid content) until developer sheet is obtained.

### EXAMPLE 2:

By treating in the same way as described in Example 1 except that instead of using ammonium phthalate in Example 1 equivalent of ammonium dicitrate is substituted developer sheet is obtained.

### COMPARISON EXAMPLE 1:

After as pigment 100 parts of heavy calcium carbonate is gently added into 100 parts of aqueous solution in which 0.5 part of sodium pyrophosphate is dissolved while stirring so that it may be well dispersed, dispersion thus obtained is added with 100 parts of 10% starch oxide aqueous solution and 10 parts (solid content) of SBR latex and further added with 30 parts of 40% papra-phenyl phenolic resin dispersion so that pH may be adjusted to 9.0 with 20% caustic soda until coating liquid is prepared. Coating liquid is coated on quality paper of 40 g/m² by means of air knife coater in such a way that the coating amount may indicate 7 g/m² (solid content) until developer sheet is obtained.

### EXAMPLE 3:

After as pigment 80 parts of heavy calcium carbonate and further 20 parts of activated clay are added into 100 parts of aqueous solution in which 0.5 part of sodium pyrophosphate while stirring so that it may well be dispersed dispersion thus obtained is added with 100 parts of 10% starch oxide aqueous solution, 10 parts of SBR latex and 30 parts of 40% para-phenyl phenolic resin dispersion and further added with 10 parts of ammonium chloride so that pH may be adjusted to 9.0 with 20% caustic soda until coating liquid is obtained. Coating liquid thus obtained is coated on quality paper of 40 g/m² by means of air knife coater in such a way that the coating amount may indicate 7 g/m² (solid content) until developer sheet is obtained.

### EXAMPLE 4 :

By treating in the same way as described in Example 3 except that instead of using ammonium chloride in Example 3 equivalent of ammonium diphosphate is used developer sheet is obtained.

### EXAMPLE 5:

By treating in the same way as described in Example 3 except that instead of using ammonium chloride in Example 3 equivalent amount of ammonium sulfate is used developer sheet is obtained.

### EXAMPLE 6:

By treating in the same way as described in Example 3 except that instead of using ammonium chloride in Example 3 equivalent amount of ammonium lactate is used developer sheet is obtained.

### COMPARISON EXAMPEL 2:

After as pigment 30 parts of heavy calcium carbonate and 20 parts are gently added into 100 parts of aqueous solution in which 0.5 part of sodium pyrophosphate while stirring and well dispersed, dispersion thus obtained is added with 100 parts of 10% starch oxide aqueous solution and 10 parts (solid content) of SBR latex and further added with 30 parts of 40% para-phenyl phenolic resin dispersion and then pH of the liquid is adjusted to 9.0 with 20% caustic soda until it is prepared as coating liquid. Coating liquid thus obtained is coated on quality paper of 40 g/m² by means of air knife coater in such a way that the coating amount may indicate 7 g/m² (solid content) until developer sheet is obtained. The test result obtained with this sheet is shown in Table 1.

Developer sheet thus obtained is laminated with the aforementioned coupler sheet and applied by pressure 96 kg/cm by means of calendering machine so that it may be allowed to form color, and then the following valuesare measured. (One hour after subjected to calendering)

o Yellowing property of developer sheet due to the effect of nitrogen oxidant:

After developer sheet is set aside in vessel containing 150 ppm of nitrogen oxidant (NOₓ) that has been generated through the method of the JIS (Japan Industrial Standard) L0855-1976 for 30 minutes, reflectivity is measured through blue filter by means of color differential meter manufactured by Nihon Denshoku Co., Ltd. It indicates that the higher the value is, the less yellowing phenomenon becomes. The test for this object has been conducted in order to test yellowing property at the time of preserving developer sheet in a dark place.

o Yellowing property of developer sheet due to irradiation of ultraviolet ray:

After ultraviolet ray is irradiated onto developer sheet by means of fadeometer manufactured by Shimazu Seisakusho for 4 hours, it is measured through blue filter by means of color differential meter manufactured by Nihon Denshoku Co., Ltd. It indicates that the higher the value is, the less yellowing phenomenon becomes.

As indicated in Table 1, as compared with developer sheet not added with ammonium salt of acid developer sheet of the present invention that is added with it is so constructed that its yellowing property due to nitrogen oxidant and yellowing phenomenon due to irradiation of ultraviolet ray are remarkably better improved than the former.

## Claims

1. A developer sheet for carbonless reproduction paper having a phenolic resin developer comprising an ammonium salt of an organic or inorganic acid as an anti-yellowing agent.

2. A sheet according to claim 1, wherein the developer further comprises an activated clay.

3. A sheet according to claim 1 or 2, wherein 1-300 parts of ammonium salt are used per 100 parts of phenolic resin, by weight.

4. A sheet according to claim 3, wherein 30-120 parts of ammonium salt are used.

5. A sheet according to any preceding claim, wherein the phenolic resin is a para-phenyl phenolic resin.
